

Jan. 27, 1959

J. HAJDU

2,871,145

PROCESS OF IMPREGNATING TEXTILE MATERIAL  
TO INCREASE ITS WEAR RESISTANCE

Filed May 21, 1954



INVENTOR  
Joseph Hajdu.

BY *Mead, Brecon, Schuyler & Kenridge*

ATTORNEYS

1

2,871,145

**PROCESS OF IMPREGNATING TEXTILE MATERIAL TO INCREASE ITS WEAR RESISTANCE**

Joseph Hajdu, Paris, France

Application May 21, 1954, Serial No. 431,603

2 Claims. (Cl. 117—139.5)

This invention relates to the treatment of textile materials such as threads, yarns, fabrics and knitted goods, and more particularly to a process of treating such materials to improve their qualities and their mechanical properties, such as resistance to wear, and to a composition suitable for use in practising said process. This application is a continuation-in-part of my prior application Serial No. 371,189, filed on July 29, 1953, now abandoned.

Known processes to improve the qualities of textiles, i. e., their resistance to wear through abrasion, their scrubbing coefficient and their mechanical properties in general, present inherent drawbacks. In the first place, their application necessitates different stages of operation, to wit, immersion of the textile in a bath, wringing the textile and drying it, all of which stages have to be repeated a number of times. The preparation of the various baths is a very delicate operation, a small variation in the composition of the bath resulting in a different effect on the textile treated. Various processes permitting a reduction in the number of baths have already been evolved but the products which went into the baths had the inconvenience of being very unstable and did not permit a prolonged use of the bath. Furthermore, the omission of coating chemicals, indispensable to achieve the result aimed at, had for direct effect the loss through washing of the qualities acquired during the treatment.

Results secured from the known treatments, though fairly satisfactory, did not achieve the necessary degree of perfection. In certain known processes, the result was a simple coating of some plastic matter on the textile, which made the textile rigid and even brittle. Another process deposited silica particles on the textile which made the feel of the fabric less desirable, or, as in the case of a process with a lesser number of baths, the desired effect was not lasting.

This invention has none of the above-mentioned drawbacks as it permits the treating of textiles through a reduced number of baths and results in a textile which presents the qualities most sought after and, at the same time, permits the production of a concentrated mixture perfectly homogeneous and stable, and which after simple dilution may be very easily applied to the textile.

It is accordingly an object of the present invention to provide a new and improved process of treating textile materials to improve their qualities and their mechanical properties in general.

It is another object of the present invention to provide such a process whereby it is possible to substantially increase the resistance to wear of a textile material.

It is a further object of the present invention to provide a new and improved composition for use in such a process.

According to a preferred embodiment of the present invention, the process consists of an immersion of the textile successively in a first bath made up of an emulsion containing at least one plastic material, one plasticizing material and possibly at least one metallic salt; then in a second bath containing an insolubilizing reagent.

2

The drawing discloses a flow diagram illustrating the process of treating textile materials in accordance with the present invention.

The treatment so applied confers upon the textile properties advantageous for the following reasons: the first bath has the effect of impregnating the textile with an emulsion of the plastic material and its plasticizing agent together with other agents which implement this impregnation by their wetting action; the second bath has the effect of breaking the emulsion and fixing the resin in situ in the fabric by precipitating the plastic material in an insoluble form within the interstices of the textile fibers. These insolubilized particles are perfectly resistant to washing, besides being supple and smooth, and thus diminish the effect of the rubbing together of the fibers by permitting the sliding of the fibers internally in the manner of ball bearings employed in mechanical constructions. In this way, instead of a coating of plastic material upon the surface of the textile, there is an impregnation of the fibers by the plastic material particles which renders the textile soft, improves its feel and, what is most important, increases its resistance to wear.

The plastic material contemplated by the present invention is a material which is insoluble in water but is emulsifiable therein and is stable to organic acids. One can use, for example, as such plastic material any synthetic or natural resin in a liquid medium. Amongst synthetic resins one will use in preference thermo-plastic materials, such as polyvinyls, polystyrene, acrylic resin, methyl methacrylate or thermo-stable materials, such as aminoplast, synthetic rubber, rubber latex, etc.

Amongst natural resins, one will use in preference those which can form an insoluble composite with aldehydes or formaldehydes or acids, as for example, natural proteins such as gelatin, casein, egg albumin, blood albumin, alginates, etc.

A textile product which is particularly resistant to washing is obtained by utilizing as the plastic material a mixture of thermoplastic resins or thermo-stable resins with proteins.

The synthetic resins may be plasticized in preparing them for the above mentioned use, and for that purpose one may use fatty materials, i. e. long chain compounds, such as paraffin, Vaseline, wax emulsions and similar hydrocarbon distillates, and natural wax emulsions. Vaseline is a trademark used by the Chesebrough Manufacturing Company, New York, New York, for its petroleum jelly.

It may be found advantageous to add wetting agents when the product is being prepared, thus permitting an easier penetration of the interstices of the fibers by the product when it is applied to textiles. Bases or alkaline salts may also be added, which will act first as stabilizers for the emulsions, then will facilitate their decomposition and insolubilization when the product is diluted.

To precipitate and insolubilize the product once it has been diluted, one can use:

- (1) Acids or metallic salts to start the precipitation.
- (2) Aldehydes to insure insolubilization.

Amongst acids, one will use in preference organic acids, such as acetic acid. Amongst metallic salts, one will use in preference acid salts of aluminum and zinc, such as borates and silicates. These organic acids and metallic salts actually break up the emulsion and cause the plastic material particles within the interstices of the textile fibers to be precipitated thereon. If one wishes at the same time to waterproof the textile, the utilization of metallic salts in place of the organic acid is advised.

The product which will constitute the first bath can be commercialized in a concentrated form and is diluted many times its volume by water when used, for example,

from 10 to 20 times or more, with the best results obtained when it is diluted with water 20 times its volume. The user therefore has the means to reproduce exactly the same bath composition which will give him the desired effect without having to handle large quantities of various liquids and compositions, as is the case with other known processes.

Furthermore, once prepared, such a bath of emulsified resins is stable and may be used over a period of time without any appreciable change occurring in its chemical composition.

The preparation of the second bath which precipitates and insolubilizes the plastic particles within the interstices of the textile fibers presents no difficulty outside of mixing the ingredients in the parts by volume specified infra.

As specific examples of resins, proteins, plasticizers, etc., suitable for the purposes of the present invention, the following are given merely for purposes of illustration and not in limitation. The term "paraffin emulsion," or any resin emulsion, which appears in the following examples is to be understood to mean a stable, aqueous dispersion of paraffin or of the particular resin. The ratios of the ingredients used in the following examples of the composition of the first bath are given in parts by weight, while the ingredients which make up the second or rinsing bath are given in parts by volume.

#### Example No. 1

A composition for a stable first bath is produced by mixing together the following ingredients in the proportions listed, which are in parts by weight, and then diluting the mixture with from 10 to 20 or more times its volume with water.

##### First bath:

|                                             |    |
|---------------------------------------------|----|
| Polyvinyl chloride emulsion                 | 45 |
| Paraffin emulsion                           | 45 |
| Dry gelatin (steeped for 24 hours in water) | 5  |
| Sodium borate                               | 5  |

The textile to be treated is first steeped in this diluted bath, preferably at 30° C., is wrung out, and then directly steeped in a rinsing bath prepared by the user and which has the following composition:

##### Second bath:

|                         |      |
|-------------------------|------|
| Water                   | 1000 |
| Acetic acid             | 20   |
| Commercial formaldehyde | 10   |

The textile is wrung out after its removal from the rinsing bath and dried at a temperature of 80° to 110° C. A textile thus treated has its mechanical properties modified as to increase its resistance to wear, and improve its rubbing coefficient.

If it is desired to also waterproof the textile, an equal quantity of aluminum acetate may be substituted for acetic acid in this rinsing bath.

Sodium silicate may be substituted for the sodium borate in the composition of the first bath and comparable results would be achieved.

#### Example No. 2

##### First bath:

|                                      |    |
|--------------------------------------|----|
| Emulsionable polyvinyl powder (pure) | 31 |
| Paraffin emulsion (concentrate)      | 45 |
| Sodium silicate                      | 5  |
| Dry gelatin                          | 1  |
| Sodium benzoate                      | 2  |
| Water                                | 16 |

##### Second bath:

|              |      |
|--------------|------|
| Water        | 1000 |
| Acetic acid  | 20   |
| Formaldehyde | 10   |

##### Second bath (for a water-repellent treatment):

|                  |      |
|------------------|------|
| Water            | 1000 |
| Aluminum acetate | 30   |
| Formaldehyde     | 10   |

The product of the first bath is diluted with water 20 times its volume to form a stable solution and the textile or fabric is steeped therein at 30° C., wrung out and then steeped in the second or rinsing bath. Depending on whether the textile or fabric is to be made water-repellent or not, one of the two examples of the second bath illustrated above may be used as the rinse bath.

Additional examples of first and second baths are illustrated infra with the composition of the concentrated mixture being diluted with water 10 to 20 or more times its volume. While baths diluted in a volume of water 10 times the volume of the composition gives satisfactory results, it has been noted that excellent results are obtained when the dilution is in the ratio of one volume of concentrated mixture to 20 volumes of water.

#### Example No. 3

##### First bath:

|                                 |    |
|---------------------------------|----|
| Paraffin emulsion (concentrate) | 45 |
| Sodium alginate                 | 10 |
| Sodium silicate                 | 5  |
| Dry gelatin                     | 1  |
| Sodium fluosilicate             | 3  |
| Water                           | 36 |

##### Second bath:

|                  |      |
|------------------|------|
| Water            | 1000 |
| Calcium chloride | 40   |
| Formaldehyde     | 10   |

##### Second bath (making the textiles water-repellent):

|                  |      |
|------------------|------|
| Water            | 1000 |
| Aluminum acetate | 30   |
| Formaldehyde     | 10   |

#### Example No. 4

##### First bath:

|                                 |    |
|---------------------------------|----|
| Paraffin emulsion (concentrate) | 45 |
| Milk caseine                    | 15 |
| Sodium silicate                 | 5  |
| Gelatin                         | 1  |
| Sodium benzoate                 | 3  |
| Water                           | 31 |

##### Second bath:

|              |      |
|--------------|------|
| Water        | 1000 |
| Acetic acid  | 10   |
| Formaldehyde | 10   |

##### Second bath (making the textiles water-repellent):

|                  |      |
|------------------|------|
| Water            | 1000 |
| Aluminum acetate | 30   |
| Formaldehyde     | 10   |

#### Example No. 5

##### First bath:

|                     |    |
|---------------------|----|
| Paraffin emulsion   | 45 |
| Egg albumen         | 10 |
| Sodium silicate     | 5  |
| Gelatin             | 1  |
| Sodium benzoate     | 3  |
| Sodium fluosilicate | 1  |
| Water               | 35 |

##### Second bath:

|              |      |
|--------------|------|
| Water        | 1000 |
| Acetic acid  | 10   |
| Formaldehyde | 10   |

##### Second bath (making the textiles water-repellent):

|                  |      |
|------------------|------|
| Water            | 1000 |
| Aluminum acetate | 30   |
| Formaldehyde     | 10   |

## Example No. 6

|                                                    |       |
|----------------------------------------------------|-------|
| First bath:                                        |       |
| Paraffin emulsion                                  | ----- |
| Blood albumen                                      | ----- |
| Sodium silicate                                    | ----- |
| Gelatin                                            | ----- |
| Sodium benzoate                                    | ----- |
| Sodium fluosilicate                                | ----- |
| Water                                              | ----- |
| Second bath:                                       |       |
| Water                                              | 1000  |
| Acetic acid                                        | 10    |
| Formaldehyde                                       | 10    |
| Second bath (making the textiles water-repellent): |       |
| Water                                              | 1000  |
| Aluminum acetate                                   | 30    |
| Formaldehyde                                       | 10    |

## Example No. 7

|                                                    |       |
|----------------------------------------------------|-------|
| First bath:                                        |       |
| Paraffin emulsion (concentrated)                   | ----- |
| Methyl methacrylate emulsion                       | ----- |
| Sodium silicate                                    | ----- |
| Gelatin                                            | ----- |
| Sodium benzoate                                    | ----- |
| Water                                              | ----- |
| Second bath:                                       |       |
| Water                                              | 1000  |
| Acetic acid                                        | 10    |
| Formaldehyde                                       | 10    |
| Second bath (making the textiles water-repellent): |       |
| Water                                              | 1000  |
| Aluminum acetate                                   | 30    |
| Formaldehyde                                       | 10    |

## Example No. 8

|                                                    |       |
|----------------------------------------------------|-------|
| First bath:                                        |       |
| Paraffin emulsion (concentrated)                   | ----- |
| Nitro-cellulose alkaline solution                  | ----- |
| Sodium silicate                                    | ----- |
| Gelatin                                            | ----- |
| Sodium benzoate                                    | ----- |
| Water                                              | ----- |
| Second bath:                                       |       |
| Water                                              | 1000  |
| Acetic acid                                        | 10    |
| Formaldehyde                                       | 10    |
| Second bath (making the textiles water-repellent): |       |
| Water                                              | 1000  |
| Aluminum acetate                                   | 30    |
| Formaldehyde                                       | 10    |

## Example No. 9

|                                  |       |
|----------------------------------|-------|
| First bath:                      |       |
| Paraffin emulsion (concentrated) | ----- |
| Latex (rubber) emulsion          | ----- |
| Sodium silicate                  | ----- |
| Gelatin                          | ----- |
| Sodium benzoate                  | ----- |
| Water                            | ----- |

## Second bath:

|    |                                                    |       |      |
|----|----------------------------------------------------|-------|------|
| 45 | Water                                              | ----- | 1000 |
| 15 | Acetic acid                                        | ----- | 10   |
| 5  | Formaldehyde                                       | ----- | 10   |
| 5  | Second bath (making the textiles water-repellent): |       |      |
| 1  | Water                                              | ----- | 1000 |
| 2  | Aluminum acetate                                   | ----- | 30   |
| 2  | Formaldehyde                                       | ----- | 10   |

30 10 Textiles, fabrics, threads, etc., treated with this two-bath process have shown a remarkable improvement in their wear resistance and rubbing coefficient. Since these treated textiles have the plastic particles disposed in the interstices of the fibers and insolubilized thereon, these particles act in the same manner as ball bearings in permitting the internal sliding of the fibers. While thus decreasing the rubbing effect on the fibers, the insolubilization of the fibers permits constant washings of the textiles without danger of removing the plastic particles therefrom.

45 20 While I have described several embodiments of my invention, I wish it to be understood that I do not intend to be restricted solely thereto and that I do intend to cover all modifications therein which would be apparent to one skilled in the art and which come within the spirit and scope of my invention.

What I claim as my invention is:

1. A process of treating textile material to increase its wear resistance comprising the steps of steeping the textile material in a first bath comprising an aqueous emulsion of an emulsifiable resin, paraffin emulsion, and gelatin, and then steeping said treated textile in a second bath comprising formaldehyde and a member selected from the group consisting of acetic acid and aluminum acetate.

35 2. A process of treating textile material to increase its wear resistance comprising the steps of steeping the textile material in a first bath comprising an aqueous emulsion of an emulsifiable resin, a plasticizing component for said resin selected from the group consisting of paraffin, petroleum jelly, and wax, gelatin, and a member selected from the group consisting of sodium borate and sodium silicate; and then steeping said treated textile in a second bath consisting of water, formaldehyde, and a member selected from the group consisting of acetic acid and aluminum acetate.

## References Cited in the file of this patent

## UNITED STATES PATENTS

|       |           |            |                |
|-------|-----------|------------|----------------|
| 10 50 | 690,868   | Menzies    | Jan. 7, 1902   |
|       | 1,476,562 | Wright     | Dec. 4, 1923   |
|       | 2,186,750 | Carter     | Jan. 9, 1940   |
|       | 2,354,662 | Bryce      | Aug. 1, 1944   |
|       | 2,357,917 | Stull      | Sept. 12, 1944 |
| 5 55  | 2,368,948 | Stallings  | Feb. 6, 1945   |
|       | 2,495,845 | Jefferson  | Jan. 31, 1950  |
|       | 2,790,736 | McLaughlin | Apr. 30, 1957  |